# EUROPEAN PATENT SPECIFICATION

(11) **EP 2 773 810 B1**
(45) Date of publication and mention of the grant of the patent: **30.12.2015**
(21) Application number: 11808953.1
(22) Date of filing: 31.10.2011
(51) Int. Cl.: D07B 1/02, D02G 3/12, H01B 5/08

(54) **COMPOSITE WIRE WITH PROTECTIVE EXTERNAL METALLIC MANTLE AND INTERNAL FIBRE**
VERBUNDDRAHT MIT EXTERNER SCHUTZUMMANTELUNG AUS METALL UND INTERNEM GEWEBE
FIL COMPOSITE COMPRENANT UN MANTEAU MÉTALLIQUE EXTERNE PROTECTEUR ET UNE FIBRE INTERNE

(43) Date of publication of application: 10.09.2014
(73) Proprietor: Redaelli Tecna S.p.A., 20135 Milano (IT)
(72) Inventor: CLERICI, Franco, I-25073 Bovezzo (BS) (IT)
(74) Representative: Bruni, Giovanni
(86) International application number: PCT/IT2011/000365
(87) International publication number: WO 2013/065074

(56) References cited:
- WO-A1-2011/094146
- GB-A- 2 187 217
- US-A- 2 458 243
- US-A- 3 091 561
- US-A- 4 084 399
- US-A1- 2010 330 365
- MCKENNA H A ET AL: "Handbook of fibre rope technology, Formation of rope structures", 1 January 2004 (2004-01-01), HANDBOOK OF FIBRE ROPE TECHNOLOGY; [WOODHEAD PUBLISHING IN TEXTILES], CAMBRIDGE : WOODHEAD ; BOCA RATON, FLA. : CRC PRESS, PAGE(S) 77 - 80, XP002514795, ISBN: 978-0-8493-2588-5

## Description

The present invention relates to a particular kind of wire comprising an outer mantle realized in metallic material and an inner portion comprising fibers, to be used autonomously or for the creation of strands or ropes, characterized by advantageous mass-resistance ratio.

An example known in the state of the art is the application n. US2010/330365**. The document** describes a strand-like material composite comprising : carbon nanotubes (CNT) yarns; a metallic component enveloping the CNT yarns to form the material composite, the material composite having a cross section, the metallic component being in the form of a matrix which spans the cross section of the material composite, wherein the CNT yarns occupy 4 to 10% by volume of the material composite.

At the state of the art, there are currently known different kinds of wire, or strands and ropes deriving therefrom, which are wholly realized in steel or other metallic material, and having undoubted advantages, such for example:
- high axial resistance;
- high capacity to bear transversal forces;
- high capacity to resist to wear phenomena;
- high corrosion resistance.

Said devices have significant drawbacks as well, such for example:
- little resistance to fire or, more generally, to high temperatures exposure, thus compromising sensibly the resistance of the metallic portions;
- high material specific weight, which inevitably leads to the overall high weight of the products realized therewith.

Just this latter aspect implies the most critical disadvantages of the known devices: in fact, in particular when vertical extended structures are referred (as for example cableways, offshore cranes, drift mines and the like), and moreover in case of very high and large structures, it is inevitable to take in consideration the weight of the single members used to bear loads.

Also in case the devices are intended for the use in water, in which case they get a hydrostatic push which leads to their overall weight to be lightened in the order of 13%, the aspect linked to the specific weight of the materials is yet significant; it is in fact clear that the effect of weight reduction of the weight linked to the floatation push is, in percentage, as greater as the specific weight of the used materials is lower. A possible solution for re-dimensioning the problems linked to the high specific weight of the construction materials lies in the possibility to use materials other than metals, as for example fibers: a constructive choice of this kind leads to the realization of a wire with highly developed mechanical features, thus guaranteeing a drastic reduction of the final product weight.

But the realization of ropes and strands entirely deriving from fiber is not possible; in fact even if the highly developed mechanical features of said materials are certain, there are as well critical points which prevent fibers from being used as sole constructive material in the realization of wires, plies and ropes, such as for example:
- problems linked to the rapid wear;
- little resistance to axial stresses;
- higher exposure to damages with respect to the metal materials;
- little detection of possible damages.

Aim of the present invention is to provide a solution which is able to overcome the main problems of specific weight, efficiency and heat resistance, peculiar to the state of the art, by means of a device which can optimize the ratio between mass and resistance thus preserving the inner fiber performance.

Another aim of the present invention is to provide a device which can be used differently in relation to the material kind in the constructive phase and in relation to the kind of treatment received.

The aim is solved by means of a new kind of composite wire, characterized by an outer mantle in metallic material and an inner portion comprising fibers and/or pultruded bars, able to conjugate the constructive advantages deriving from the use of these latter, and avoiding as well the problems in terms of wear exposure and damages by means of a protective coating mantle.

These and other characteristics of the invention will be better highlighted in the following description of a preferred embodiment, which refers to the drawings 1/3, 2/3 and 3/3, in which;
- figure 1 shows the section of a preferred embodiment of a strand comprising several wires, each wire characterized by an outer mantle in metallic material and an inner portion comprising fibers;
- figure 2 shows the section of a preferred embodiment of a strand comprising several wires, each wire characterized by an outer mantle in metallic material, a first inner portion comprising fibers and a second inner portion represented by a pultruded bar, the whole being after subjected to a compacting process;
- figure 3 shows the section of a preferred embodiment of a rope, made up of strands positioned in turn each strand characterized by several wires, each wire having an outer mantle in metallic material and an inner portion comprising fibers;
- figure 4 shows a tridimensional view of a preferred embodiment of a wire, characterized by a linear outer mantle in metallic material and an inner portion comprising fibers arranged in parallel bundles;
- figure 5 shows a tridimensional view of a preferred embodiment of a wire, characterized by a linear outer mantle in metallic material, a first inner portion comprising fibers arranged in parallel bundles and a second inner portion comprising a pultruded bar;
- figure 6 shows a tridimensional view of a preferred embodiment of a wire, characterized by an outer mantle in linear metallic material and an inner portion comprising fibers twisted around each other;
- figure 7 shows a tridimensional view of a preferred embodiment of a wire, characterized by a helical outer mantle in metallic material and an inner portion comprising fibers arranged in parallel bundles.

As yet stated, object of the present invention is a particular and innovative kind of composite wire 10, having an outer mantle 1 in metallic material with protective functions, and an inner portion comprising fibers 2, able to overcome the problems linked to the specific weight and little resistance to high temperatures and pressures at the state of the art, and characterized by an advantageous mass-resistance ratio.

By using an outer mantle 1 realized in metallic material it is possible to solve the damaging and little resistance to transversal load problems, peculiar to the fibers 2.

Likewise, the introduction of an inner portion comprising fibers 2 and/or pultruded bars 3 makes it possible to obtain sensible advantages, as for example:
- sensible reduction in the specific weight of the construction material (for example in a possible preferred embodiment of a wire 10, which is 40% made up of steel and in the remaining 60% made up of highly resistant fibers with specific weight approximately 1,4, there results a final device with a specific weight equal to 50% of the steel one, in the air, or 40% in water);
- higher fire resistance;
- higher resistance in case of high temperatures, above all in the case the composite wires 10 containing an inner core in glass fiber 3;
- possibility to delay the inner temperature increase of the wire 10 in case of prolonged exposure to high temperatures;
- contribution to the whole load capacity.

Figures 4 to 7 represent tridimensional views of preferred embodiments of the invention, some of them being made up of only two layers, i.e. a linear (figures 4 and 6) or helical (figure 7) outer mantle l in metallic material, and an inner portion comprising fibers 2 arranged in parallel bundles (figures 4 and 7) or twisted around each other (figure 6), the other one comprising also another inner portion represented by a pultruded bar 3 (figure 5). The use for example of a bar in glass fiber 3 as innermost portion of the wire 10 (figures 2 and 5) contributes sensibly to implement its features of resistance and of high temperatures and transversal pressures bearing.

Clearly, the axial and transversal, dimensional and resistance features as well as the elasticity of the composite wire 10 can be differently modulated using metal outer mantle 1 with different resistance, diameter or thickness, possibly helically wound as well, in turn in variable combination with different combinations of fibers 2 and/or pultruded bars 3, which can be used in parallel or helical bundles (figures 4 to 7) as well.

Also the external features of corrosion resistance of the wire 10 can be differently determined by choosing materials for the realization of the outer mantle 1, as well as the respective superficial finishing with the longitudinal edges to be welded; in this last case, considering all the other features for certain, an increase of the torsional resistance of the wire 10 can be detected.

Finally, also the different mode of treatment and impregnation (resins, lubricants, buffers) of the fibers 2 contributes to different connotations of the used material.

As yet stated, said composite wires 10 can be used autonomously, as long as they are provided with specific ends or connections, or they can constitute portions of the bundles, strands 12 (figure 1), these ones also being compacted (figure 2), or of ropes 13 made up of said strands 12 (figure 3).

With these features in terms of lightness and resistance, peculiar to the device object of the invention, it is clear that this one is mainly intended for the use in all the fields where the aspect linked to the specific weight of the various elements is particularly important (offshore deep sea, drift mines, aeronautics, architecture): said uses represent however a purely preferred possibility of use and do not exclude other possible and suitable uses.

In particular, it is to be highlighted that said wire can be also used as vehicle for conducting electric energy, using fibers 2 coated with an aluminum mantle 1 : such a possibility would allow to solve many problems linked to the weight and the high thermal expansion of the solutions currently available, which are mainly characterized by the use of steel and aluminum cables.

What described represents only some preferred embodiments of the invention; it is intended that modifications and/or variations of the same are possible, without departing from the aims of the present invention, as defined by the following claims.

## Claims

1. Composite wire (10) having a contained specific weight and high traction resistance, suitable to be used autonomously or as part of bundles, strands (12) or ropes (13) formed therefrom, comprising:
- at least an outer mantle (1) in metallic material with protective function;
- at least an inner portion comprising fibers (2), **characterized in that** the outer mantle (1) is a metallic, encasing tube which is welded at the longitudinal edges.

2. Composite wire (10) according to claim 1, **characterized in that** said inner portion comprising fibers (2) is an inner layer containing a further fibrous portion (3) therein.

3. Composite wire (10) according to claim 2, **characterized in that** said further portion is a pultruded bar (3).

4. Composite wire (10) according to claim 1, **characterized in that** the edges extend parallel to the longitudinal axis of the composite wire (10).

5. Composite wire (10) according to claim 1, **characterized in that** the edges run helically.

6. Composite wire (10) according to any one of claims 1 to 5, **characterized in that** the fibers (2) and/or the pultruded bars (3) are arranged parallel to the longitudinal axis of the composite wire (10).

7. Composite wire (10) according to any one of claims 1 to 5, **characterized in that** fibers (2) and/or the pultruded bars (3) are twisted around each other.

8. Strand (12) for ropes (13) comprising a plurality of composite wires (10) according to anyone of claims 1 to 7.

9. Rope (13) comprising one or more strands (12) according to claim 8.

10. Use of the composite wire (10) according to claim 1, for electric energy conduction, wherein the outer mantle (1) for protecting the fibers (2) is realized in aluminum.

## Patentansprüche

1. Verbundkabel (10) mit einem begrenzten spezifischen Gewicht und einer hohen Zugfestigkeit, das geeignet ist, autonom betrieben oder als Teil von damit gebildeten Bündeln, Streifen (12) oder Seilen (13) verwendet zu werden, umfassend:
- zumindest eine äußere Hülle (1) aus metallischem Material mit einer Schutzfunktion;
- zumindest einen Innenteil mit Fasern (2), **dadurch gekennzeichnet, dass** der Außenmantel (2) aus einem Metallrohr besteht, das an den Längskanten verschweißt ist.

2. Verbundkabel (10) nach Anspruch 1, **dadurch gekennzeichnet, dass** der besagte innerer Teil Fasern (2) in einer inneren Schicht aufweist, die intern einen zusätzlichen faserförmigen Teil (3) aufweist.

3. Verbundkabel (10) nach Anspruch 2, **dadurch gekennzeichnet, dass** der besagte zusätzlicher Teil eine Zugextrudierte Stange (3) ist.

4. Verbundkabel (10) nach Anspruch 1, **dadurch gekennzeichnet, dass** sich die Kanten parallel zur Längsachse des Verbundkabels (10) erstrecken.

5. Verbundkabel (10) nach Anspruch 1, **dadurch gekennzeichnet, dass** sich die Ränder schraubenförmig erstrecken.

6. Verbundkabel (10) nach einem der Ansprüche 1 bis 5, **dadurch gekennzeichnet, dass** die Fasern (2) und/oder die Zugextrudierten Stangen (3) parallel zur Längsachse des Verbundkabels (10) angeordnet sind.

7. Verbundkabel (10) nach einem der Ansprüche 1 bis 5, **dadurch gekennzeichnet, dass** die Fasern (2) und/oder die Zugextrudierten Stangen (3) aneinander gedreht werden.

8. Bündel (12) für Seile (13) mit einer Vielzahl von Verbundkabeln (10) nach einem der Ansprüche 1 bis 7.

9. Seil (13), umfassend ein oder mehrere Bündel (12) nach Anspruch 8.

10. Verwendung des Verbundkabels (10) nach Anspruch 1 zur Leitung einer elektrischen Energie, wobei der äußere Mantel (1) aus Aluminium besteht, um die Fasern (2) zu schützen.

## Revendications

1. Câble composite (10) ayant un en poids spécifique contenu et une résistance élevée à la traction, apte à être actionné de manière autonome ou en tant que partie de faisceaux, des bandes (12) ou de cordons (13) formés par celui-ci, comprenant:
- au moins une enveloppe extérieure (1) en matériau métallique avec une fonction de protection;
- au moins une partie interne comprenant des fibres (2), **caractérisé en ce que** l'enveloppe extérieure (2) est un tube externe métallique qui est soudé sur ses bords longitudinaux.

2. Câble composite (10) selon la revendication 1, **caractérisé en ce que** ladite partie intérieure comprend des fibres (2) dans une couche interne contenant une partie supplémentaire fibreuse (3) à son intérieur.

3. Câble composite (10) selon la revendication 2, **caractérisé en ce que** ladite partie supplémentaire est une tige (3) extrudée par traction.

4. Câble composite (10) selon la revendication 1, **caractérisé en ce que** les bords sont développés parallèlement à l'axe longitudinal du câble composite (10).

5. Câble composite (10) selon la revendication 1, **caractérisé en ce que** les bords sont développées dans le sens hélicoïdal.

6. Câble composite (10) selon l'une quelconque des revendications 1 à 5, **caractérisé en ce que** les fibres (2) et/ou les tiges (3) extrudées par traction sont disposées parallèlement sur l'axe longitudinal du câble composite (10).

7. Câble composite (10) selon l'une quelconque des revendications 1 à 5, **caractérisé en ce que** les fibres (2) et/ou les tiges (3) extrudées par traction sont entraînés en rotation l'une autour de l'autre.

8. Faisceau (12) pour des câbles (13) comprenant une pluralité de câbles composites (10) selon l'une quelconque des revendications 1 à 7.

9. Corde (13) comprenant un ou plusieurs faisceaux (112) selon la revendication 8.

10. Utilisation du câble composite (10) selon la revendication 1, pour la conduction d'énergie électrique, dans lequel l'enveloppe extérieur (1) afin de protéger les fibres (2) est en aluminium.
